

Nov. 25, 1969

W. TURTON ET AL

3,479,710

TEXTURED TEXTILE MATERIAL

Filed Dec. 13, 1967



Fig. 1



Fig. 2



Fig. 3

INVENTORS  
WALTER TURTON  
CHARLES MAZZONE  
BY  
*John Paul Coenar*  
ATTORNEY

**1**

3,479,710

**TEXTURED TEXTILE MATERIAL**

Walter Turton, Stamford, Conn., and Charles Mazzone, Dover, N.J., assignors to J. P. Stevens & Co., Inc., New York, N.Y., a corporation of Delaware  
Filed Dec. 13, 1967, Ser. No. 690,288  
Int. Cl. D02g 3/22; D02j 1/22  
U.S. Cl. 28—72

4 Claims

**ABSTRACT OF THE DISCLOSURE**

A method and apparatus for texturizing a textile material wherein the material is mechanically deformed to introduce flattened segments of reduced cross-sectional areas along the length of the yarn whereby a high degree of residual shrinkage is maintained in said yarn. This textured yarn exhibits an ability to cause a high degree of stitch distortion when knit in combination with an untextured yarn into a tricot fabric.

This invention relates to the texturizing of thermoplastic textile yarn. One aspect of the present invention relates to a method of processing thermoplastic textile yarn to produce filaments thereof having variegated cross-sectional shapes at various intervals along the length thereof. Another aspect of this invention relates to an apparatus for distorting a textile yarn at various intervals along the length thereof. Yet another aspect of this invention is to produce a textured thermoplastic synthetic linear high polymer yarn such as polycaproamide (nylon 6) for use in tricot knits, hosiery, wovens, and other types of fabrics.

In order to impart certain desirable properties to continuous man-made filament yarn it has become common practice to texturize or loft the same. Textured yarn possesses greater bulkiness, better heat insulating power and other improved properties while still retaining many of the desirable characteristics of spun yarn. These properties were achieved by artificially cramping the man-made yarns in order to simulate the bulkiness of certain wool fibers whose bulkiness is a direct consequence of the kinked or curled character of wool.

One method of considerable commercial significance for producing textured yarn involves the steps of introducing textile material in a substantially tensionless state between a set of opposed surfaces whose alternate depressed and raised areas are engaging under an applied pressure and which engage the material and each other so that the material as a result of the tensionless feed zigzags laterally just prior to being gripped and crimped. This method is described in a patent, No. 3,345,718, issued on Oct. 10, 1967, to Hollihan et al. and assigned to J. P. Stevens & Co., Inc.

Another method of considerable commercial significance for producing textured yarn involves the steps of hot-drawing substantially undrawn thermoplastic continuous filament yarn and immediately thereafter simultaneously cooling and deforming the yarn by passing same between a pair of intermeshing gears.

Another method of considerable commercial importance produces a twist-curved yarn having a lively stretch. Ordinarily, twist-curved textured yarn is made by a 3-step process. In the first step, the yarn is twisted a desired amount. While in the twisted condition, the yarn is heat-set during the second step. That is, the yarn is heated and cooled while twisted so as to render the yarn dimensionally stable until again heated to or above the setting temperature. Finally, the yarn is untwisted. The twist imparted and set in the yarn can be a true twist or a false twist.

Still another method of considerable commercial im-

**2**

portance utilizes the well-known stuffing box technique to induce substantially permanent crimp into the yarn. The yarn is characterized by sharp elbows between the arms of the crimps induced therein.

It has also been known to produce a textured continuous filament yarn by knitting the yarn into fabric, heat-setting the fabric and unravelling the fabric. In addition, hot gas jet processes are known for texturizing filament yarn. All of the prior art processes are concerned with imparting a crimp to the yarn being treated.

The subject invention is not concerned with imparting a crimp into the yarn in order to increase its bulkiness but rather the subject invention relates to a process for flattening the yarn at various intervals along the length thereof. Moreover the above described prior art methods for producing crimped yarn generally result in a product which has a markedly reduced shrinkage. Since the yarn is in a relaxed condition, there is nothing to prevent the yarn from shrinking to its fullest extent. Even though the yarn may be subsequently straightened under tension for purposes of packaging or other textile operations, it will never regain its normal shrinkage. For example, normally drawn nylon 6 has a shrinkage of greater than 8% and usually between 13 and 15%, whereas similar yarn which has been given a heat treatment while relaxed will have a shrinkage value between 0% and 5%. Yarns that have been subjected to a knit-set treatment or crimped in a stuffer box are heated in a substantially tension-free condition to set the crimp in the yarn at which point a very low shrinkage results.

The term "shrinkage" as used throughout the specification and claims is intended to mean the actual shortening of the yarn along its actual length, which phenomena is the result of exposure to heat in a relaxed condition such as by immersion in boiling water or steam. The term "residual shrinkage" employed hereinafter means that after being treated the yarn is still able to be further shortened by a subsequent heat treatment.

The term "yarn" is used to include filaments, tows, slivers, rovings, ribbons, and the like and relates to both monofilament and multifilament yarns.

One object of this invention is to provide textured yarn having a variegated cross-sectional shape along the length thereof;

Another object of this invention is to vary the bending modulus along the length of said yarn;

Another object of this invention is to vary the modulus or flex of thermoplastic yarns at various intervals along the length thereof;

Yet another object of this invention is to produce a permanently intermittently flattened synthetic linear high-polymer yarn that may be collected in package form;

Still another object of the present invention is the production of a synthetic linear high-polymer yarn that possesses at least 5% residual shrinkage.

A still further object of the present invention is to provide a process for treating synthetic linear high-polymeric yarn to produce intermittent permanent flattening along the length thereof;

A still further object of the present invention is to provide a process for permanently distorting synthetic linear high-polymeric yarn which is readily adaptable to existing yarn-treating systems and thereby avoid the addition of separate operating steps;

A still further object of this invention is the provision of a yarn-treating process which insofar as known functions at relatively high or low operating speeds although the quality of the yarn improves as the speed increases and which is not limited in performance to prolonged exposure or dwell time between the yarn and the source of heat at the flattening point;

Other objects and many of the attendant advantages of this invention will be readily appreciated as the same becomes better understood by reference to the following detailed description which is to be considered in connection with the accompanying drawings wherein:

FIG. 1 is an elevational schematic view of one embodiment of an apparatus according to the invention;

FIG. 2 is an enlarged detail showing the engagement of the rolls for deforming the textile material according to this invention; and

FIG. 3 is an enlarged view in perspective of segments of textile products produced in accordance with the invention.

One of the purposes of producing a yarn, having the deformation described herein at determined intervals is to provide effects in fabrics when said yarn is knitted or woven in combination with untextured yarns. For example, the yarn of the present invention, when combined with normal yarn in a tricot fabric, produces a pleasing appearance and hand by virtue of the distortion in the fabric surface. These effects in the fabric are caused by a loop distortion produced during the knitting cycle due to the varying modulus of bending brought about by variation in the cross-sectional shape of the textured yarn due to the flattening of the yarn at regular or irregular intervals. Moreover, a residual shrinkage of at least 5% remaining in the treated yarn will assist in drawing the companion yarn out of its normal stitch pattern.

In the aforementioned texturizing processes, the textured yarns treated cannot accomplish this effectively since their shrinkage after processing is very low, namely, from 1 to 2%. The yarn of the present invention having both a flattening as opposed to a crimped configuration as well as a high residual shrinkage produces a novel and desirable result in tricot fabric because of the convolutions of the yarn itself and also of the distortion of the companion yarn from a normal stitch pattern. The second effect improves as the shrinkage value increases.

Briefly the method of this invention comprises the steps of flattening a softened thermoplastic yarn to introduce segments of reduced cross-sectional area into the yarn; correlative controlling the pressures and temperatures to which the yarn is subjected in order to permanently distort the yarn while maintaining a residual shrinkage of at least 5% in said flattened yarn; and collecting the yarn under a controlled tension in an orderly manner in compact package form.

According to this invention previously drawn synthetic thermoplastic yarns that have little or no distortions are pressed between two surfaces one of which is engraved while the other of which is substantially smooth. The yarn is in a softened or plasticized condition to permanently impress into the fibers flattened distortions that are preferably closely spaced.

A textile product in accordance with this invention can be manufactured from a wide variety of material. For example the textile product may be proteinaceous material, cellulosic material, synthetic thermoplastic polymeric material, thermosetting polymeric material, and the like. Illustrative of such materials are the cellulosic fibers, cellulosic acetate fibers, the polyamides, polyesters, acrylics, and the like.

The preferred form of this invention is to flatten at various intervals along the length thereof a continuous monofilament yarn between two nip rolls the upper roll of which is serrated around the periphery thereof while the lower roll is substantially smooth around the periphery thereof. The faces of the nip rolls are brought into close contact under a pressing relation with the monofilament yarn by means of weights, spring pressure, hydraulic pressure, or the like. Moreover the flattened distortions present a substantially constant distribution pattern throughout any given length of the monofilament yarn prepared by the process of the invention as set forth

more fully hereinbelow. However, it is possible to produce flattenings at random along the length of the monofilament yarn in cases where special effects are desired.

The number of flattenings per given linear inch varies in the range from 20 to 62 and preferably from 25 to 45. If the frequency in the number of deformations is maintained within this range, a textured yarn is produced capable when knitted into a tricot fabric with an untextured yarn of providing the said fabric with a pronounced crepe effect. Moreover it is not intended to confine this invention to lengths of the textured yarns being left in original form. Deformation of the full filament length is permissible so long as there are sufficient variations, which may vary or not vary in size, in the yarn to effect the flex modulus thereof. The denier size of the filaments must also be coordinated with the deformation frequency because as the denier size is increased the number of deformations per unit linear length must also be increased to provide a suitable textured yarn. In our preferred embodiment we employed 15-denier monofilament yarn.

After flattening of the textile material between the surfaces takes place, the material is removed while being maintained under controlled tension. The product has a substantial proportion of the flattening imparted thereto retained substantially permanently.

Generally the fibrous textile material is removed from between the opposed surfaces in a substantially tensionless state. It may be cooled by ambient temperature or it may be positively cooled while being removed from between the opposed surfaces.

The material being treated is processed at a temperature and pressure at least sufficient to permit it to undergo permanent deformation and prevent excessive shrinkage in the fiber. The temperatures and pressures are correlated to insure that the textured fiber maintains a residual shrinkage of at least 5%.

Where a positive heating step is utilized, the material to be treated can be raised to an elevated temperature by any suitable means either before it passes between the surfaces which deform it or while it is physically present between the surfaces and undergoing deformation.

The particular temperature employed in the treatment of a particular textile filamentary material depends upon the characteristics of the material itself. For example, certain types of proteinaceous materials are readily processed at room temperature, that is, at about 20° C. On the other hand, a synthetic material such as nylon is processed at a temperature of from between 150 to 180° C. This process can be carried out at lower temperatures than the crimping procedure set forth hereinabove.

In carrying out the process of this invention, the textile material being treated is deformed between the opposed surfaces at a wide variation of applied pressures.

The particular amount of pressure should be at least sufficient to insure that the material passing between the opposed surfaces is made to produce flattening at various intervals along the length of the fiber. At the same time the material should not have so much pressure applied thereto that it is physically damaged by contact between the surfaces. Generally speaking, applied pressures in a range of from 240 to 400 pounds per linear inch of the roll is sufficient in most cases to achieve the desired object. On the other hand it is to be noted that the most suitable pressure necessary for processing of any particular fiber is readily determinable and is limited mainly by physical limitations of the apparatus or physical limitations of the fibrous material itself.

In carrying out the practice of the invention it should also be noted that positive means for setting the material being treated are preferably, although not necessarily, utilized. As pointed out hereinabove such means may include raising the fibrous material to an elevated temperature but also may include pretreatment with a chemical setting agent or the like.

Any suitable chemical setting agent for the particular fibrous material being processed can be used. Examples

of suitable chemical setting agents for keratin based fibers are reducing agents, alkaline reducing agents, thiols such as thioglycollic acid and saturated steam at elevated pressures. For other proteinaceous fibers such as silk, high temperature steam and any of the conventional tanning chemicals as well as formaldehyde may be used. For cellulosics, the setting agents could be drawn from any of the chemical groups such as formaldehyde, urea formaldehyde, melamine formaldehyde, and other such thermo-setting agents or chemicals. In general any chemical which is able to supply permanent crosslinking either by covalent or by any other type of permanent bonding is suitable. Thermoplastic fibers may be presoftened either by heat or the use of volatile plastisizers which would be evaporated off during the setting operation.

With one's attention now being directed to the drawings, further elucidation of the present invention will be given. There is shown in FIG. 1 an apparatus generally designated as 10 which is suitable for treatment of textile material, in this case illustrated as fibers, in accordance with the invention. In this embodiment there is depicted a beam 11 on which is wound a large number of ends of a monofilament textile material, in this case illustrated as fibers, in accordance with the invention. Beam 11 is supported by journal means, not shown, and is free-running but provided with a friction drag or other suitable device to provide uniform tension in the fibrous textile material on the beam.

The fibrous textile material 13 passes through a reed 15 supported by means not shown.

The material 13 then passes between a set of grooved surfaces illustrated as a pair of rolls 19 and 21. Although only two surfaces are illustrated in this embodiment, the number of opposed surfaces may be greater than two. At least one of the rolls, preferably the one placed in the upper position 19, is provided with an engraved surface having a surface configuration which is designed to impart a flattening at various intervals along the length of the textile material 13 passing between the two surfaces. In order to obtain a flattening as opposed to a crimping effect, it is critical that the bottom roll 21 has a smooth unembossed surface. The nature of the composition of rolls 19 and 21 is not critical but should be of a material that can withstand heat and pressure in order to prevent either of them from wearing excessively.

Drive roll 19 is rotated by means not shown and roll 21 is driven as a result of the frictional force resulting from the pressure contact with roll 19.

One or both of the rolls may be heated by conventional means such as oil circulating inside the roll or rolls to facilitate the deformation of the material 13 between the rolls.

The take-up assembly, generally designated as 23 comprises rolls 25 and 27 and is capable of maintaining the fibrous textile material 13 under controlled tension until it is cooled sufficiently to retain substantially permanently the flattening configuration imparted thereto. Both rolls 25 and 27 are driven by means not shown. Any suitable take-up assembly may be used for this purpose; moreover the take-up rolls may comprise a set of rolls which can be greater than two in number if desirable. In addition it is to be noted that either one or both of the take-up rolls 25 and 27 can be utilized to provide positive cooling means for cooling the textile material being processed. It should be further understood, however, that the textile material being treated may be cooled sufficiently to achieve substantially permanent configuration of the deformation therein solely as a result of ambient heat exchange. Therefore rolls 25 and 27 would not have to be adapted for cooling purposes.

Alternative methods of cooling are also possible such as passing the material through an atmosphere which is maintained at a low ambient temperature. Regardless of the particular method of cooling utilized, the cooling should be accomplished before the yarns are exposed to

forces which would tend to remove the flattening imparted thereby by rolls 19 and 21.

The textured yarn is wound onto beam 30 after passing from the take-up assembly 23.

With reference to FIG. 2, grooves 29 in roll 19 are helical and are at an angle of approximately 25 degrees with the axis of roll 19. The grooves 29 are separated by land areas 32. The helical configuration is used to avoid pattern repeats in a fabric woven or knitted from material processed in accordance with the invention. However, for the purposes of this invention, it is to be appreciated that the angle of the grooves is not critical and that in fact the engraved roll may have grooves which are vertical to the horizontal.

Since this is not a crimping operation but rather a flattening of the fiber at various intervals, the depth of grooves 29 are dependent in part on the spacing thereof. That is to say, the maximum depth is limited by the requisite land area configuration needed to withstand the pressures necessary for the flattening operation. The permissible depth of the grooves may range from 0.004 inch to about 0.010 inch. Naturally it is desirable to remove any and all sharp edges so as to avoid any possibility of cutting the yarn being treated.

With respect to the selection of diameters for rolls 19 and 21, the embodiment shown in FIG. 1 depicts substantially equal diameters. However, the bottom roll can be of larger diameter than the top roll.

FIG. 3 shows a yarn 31 which has been texturized according to the process described hereinabove.

The following examples are offered to illustrate the principle of this invention. Nylon 66 yarn (polymer of adipic acid and hexamethylenediamine) was treated according to the teaching of this invention.

#### EXAMPLE 1

An apparatus similar to that shown in FIG. 1 was used, with roll 19 having 62 grooves per inch, equally spaced, and positioned at an angle of 26° to the axis of rotation of the rolls. The grooves in roll 19 have a depth of 0.008 inch. There was no cooling other than natural ambient heat exchange. Roll 19 was composed of steel and roll 21 was composed of nylon.

A sheet of 15/1 polyhexamethylene adipamide (type 66 nylon) containing 588 ends was flattened at a linear speed through rolls 19 and 21 at 150 feet per minute.

It was found that suitably flattened yarn was produced with a pressure of 180 pounds per linear inch when roll 19 was heated to 370° F. This yarn retained 5.5% of its residual shrinkage.<sup>1</sup>

This textured yarn having 28 needles per inch when knit in a tricot machine along with an untextured 20/7 nylon 66 yarn produced a tricot fabric exhibiting a pleasing appearance and hand by virtue of the distortion of the stitch formation.

#### EXAMPLE 2

An apparatus similar to that shown in FIG. 1 was used, with roll 19 having 40 grooves per inch, equally spaced, and positioned at an angle of 45° to the axis of rotation of the rolls. The grooves 29 in roll 19 had a depth of 0.008 inch. There was no cooling other than natural ambient heat exchange. Rolls 19 and 21 were composed of steel and nylon respectively.

A single end type 66 nylon 15/1 monofilament yarn was flattened at a linear speed through rolls 19 and 21 at 150 feet per minute.

It was found that suitably flattened yarn was produced with a pressure of 180 pounds per linear inch when roll 19 was heated to 370° F. This yarn retained 5.5% of its residual shrinkage.<sup>1</sup>

This textured yarn when knit as in Example 1 produced a tricot fabric exhibiting a pleasing appearance and hand by virtue of the distortion of the stitch formation.

See footnote<sup>1</sup> at bottom of Column 7.

7  
EXAMPLE 3

An apparatus similar to that shown in FIG. 1 also heated with roll 19 having 25 grooves per inch, equally spaced and positioned at an angle of 45° to the axis of rotation of the rolls. The grooves 29 in roll 19 had a depth of 0.011 inch. There was no cooling other than natural ambient heat exchange. Rolls 19 and 21 were composed of steel and nylon respectively.

A single end type 66 nylon 15/1 monofilament yarn was flattened at a linear speed through rolls 19 and 21 at 10 150 feet per minute.

It was found that suitably flattened yarn was produced with a pressure of 120 pounds per linear inch when roll 19 was heated to 290° F. This yarn retained 8.0% of its residual shrinkage.<sup>1</sup>

## EXAMPLE 4

An apparatus similar to that shown in FIG. 1 also heated with roll 19 having 25 grooves per inch, equally spaced and positioned at an angle of 45° to the axis of 20 rotation of the rolls. The grooves 29 in roll 19 had a depth of 0.011 inch. There was no cooling other than natural ambient heat exchange. Rolls 19 and 21 were composed of steel and nylon respectively.

A single end type 66 nylon 15/1 monofilament yarn was flattened at a linear speed through rolls 19 and 21 at 25 150 feet per minute.

It was found that suitably flattened yarn was produced with a pressure of 120 pounds per linear inch when roll 19 was heated to 325° F. This yarn retained 7.8% of its 30 residual shrinkage.<sup>1</sup>

## EXAMPLE 5

An apparatus similar to that shown in FIG. 1 also heated with roll 19 having 25 grooves per inch, equally spaced and positioned at an angle of 45° to the axis of rotation of the rolls. The grooves 29 in roll 19 had a depth of 0.011 inch. There was no cooling other than natural ambient heat exchange. Rolls 19 and 21 were composed of steel and nylon respectively.

A single end type 66 nylon 15/1 monofilament yarn was flattened at a linear speed through rolls 19 and 21 at 40 150 feet per minute.

It was found that suitably flattened yarn was produced with a pressure of 120 pounds per linear inch when roll 19 was heated to 365° F. This yarn retained 5.0% of its 45 residual shrinkage.<sup>1</sup>

<sup>1</sup> Single end Shrinkage:

## SCOPE

This method has been developed by J. P. Stevens to test the shrinkage of an individual end of filament yarn removed from a woven or knitted fabric.

## PROCEDURE

- (1) Loops 75 to 100 cm. of yarn. Tie ends together.
- (2) Hang yarn on vertical meter stick (attached to wall) that has a peg at top which serves as a hook for yarn.
- (3) Attach .1 gm./denier×2 (number of ends in loop) to 50 yarn. Record reading A.
- (4) Remove weight and boil off (210-212° F.) in cheese cloth. Time 30 minutes.
- (5) Dry for two hours in a steam heated oven (closed coil) 55 110-120° F.
- (6) Hang on vertical meter stick and repeat Step 3. Record as length B.

Calculation:  $\frac{A-B}{A} \times 100 = \text{percent shrinkage}$

5 The permanency of the distortions in the yarn flattened according to the conditions described in Examples 3, 4 and 5 was not affected.

Obviously many modifications and variations of the present invention are possible in the light of the above teachings. It is therefore to be understood that within the scope of the appended claims the invention may be practiced otherwise than as specifically described herein.

15 What is claimed is:

1. A process for texturizing a monofilament thermoplastic yarn comprising the steps of flattening a softened previously drawn monofilament thermoplastic yarn to introduce segments of reduced cross-sectional areas into the yarn whereby said yarn exhibits a variation in bending modulus along the length thereof; correlative controlling the pressures and temperatures to which the yarn is subjected in order to effect permanent distortion of the yarn while maintaining a residual shrinkage of at least 5% in said flattened yarn, and collecting the textured yarn under a controlled tension so as to eliminate any further drawing thereof in an orderly manner in compact package form, whereby a yarn having varigated cross-sectional shapes of uniform consistency located at predetermined intervals along the length thereof is produced.

2. A process according to claim 1 wherein the number of flattenings per given linear inch varies in the range from 20 to 62.

35 3. A process according to claim 1 wherein the yarn is treated at a temperature ranging from 150 to 370° F.

4. A process according to claim 1 wherein a polyhexamethylene adipamide monofilament yarn is texturized.

40

## References Cited

## UNITED STATES PATENTS

- 2,044,135 6/1936 Taylor.  
2,975,474 3/1961 Smith.  
3,069,726 12/1962 Adams.  
3,116,197 12/1963 Kasey.

## FOREIGN PATENTS

- 50 1,462,511 11/1966 France.

55 JAMES KEE CHI, Primary Examiner

U.S. Cl. X.R.

28—1; 57—140